

## UNITED STATES PATENT OFFICE

2,605,183

## HETERO CYCLIC ALKYLAMINES AS ACCELERATORS FOR PHOTOGRAPHIC DEVELOPERS

Ivy V. Runyan, Binghamton, N. Y., assignor to  
General Aniline & Film Corporation, New York,  
N. Y., a corporation of Delaware

No Drawing. Application November 16, 1949,  
Serial No. 127,779

12 Claims. (Cl. 95—88)

1

This invention relates to photographic developers and particularly to nuclear aminoalkyl substituted heterocyclic compounds as accelerators for photographic developers.

It is well known that various amines, such as primary and secondary alkyl and alkylene amines containing from 3 to 7 carbon atoms, may be added to photographic black and white and color developing solutions for the purpose of increasing the rate of development. In other words, these amines accelerate the development so as to cause the developing agent to form the image (silver or color image) more rapidly than is possible without the presence of such amines.

Although developing solutions containing such amines cut the developing time to 12–15 minutes, such period is still unsatisfactory where large scale operations are involved, as in commercial processing where time is of the essence.

It is also known that nitrogenous heterocyclic bases, such as piperidine, pyrrolidine, morpholine, piperazine, lysidine and the like, which, when present in color forming photographic developers in an amount ranging from about 0.5 gram to 4 grams per liter, make it possible to obtain images having a harmonious gradation, reduced contrast, and satisfactory brilliance. While these bases energize weak color forming photographic developers to the extent that pictures of improved appearance are obtained, they do not, however, permit a reduction in development time, nor do they permit the development of pictures having an overall increased contrast. Moreover, the use of these heterocyclic bases in color developers may lead to skin irritations and sometimes eruptions when color development of the film is done with bare hands.

It is, therefore, an object of the present invention to provide a black and white and color developer having an increased rate of development so that developing time is substantially decreased to less than half of the normal time without loss of contrast and speed.

A further object is to provide nuclear aminoalkyl substituted heterocyclic compounds as accelerators for photographic developers which are less toxic than the alkylamines and heterocyclic bases of the prior art.

Other objects will appear hereinafter.

The foregoing objects are accomplished by adding a nuclear aminoalkyl substituted heterocyclic compound to the usual black and white developer and to a color forming developer in which a primary aromatic amine is used as the developing agent. It has been found that in developing

2

color images in multicolor photographic layers containing color formers fast to diffusion, as disclosed in United States Patents 2,173,612, 2,179,228, 2,179,234, 2,179,238–9, 2,179,244, 2,186,719, 2,186,851, 2,186,852, 2,186,732–3–4, 2,186,849, 2,200,306, 2,280,722, 2,292,575, 2,303,928, and 2,307,399, with a color developer containing a nuclear aminoalkyl substituted heterocyclic compound, the developing time is cut from 20–30 minutes to 2–10 minutes. All of the layers are simultaneously developed and the dye images formed are of excellent quality.

The developing time with black and white developers, for instance, solutions of hydroquinone and Metol (p-methylaminophenol sulfate) and the like, is also cut by more than half without causing fog when such solutions contain a nuclear aminoalkyl substituted heterocyclic compound.

The accelerators employed in accordance with the present invention are heterocyclic compounds containing an aminoalkyl group of not more than 3 carbon atoms substitutes (i. e., for a hydrogen atom) in the nucleus of such compounds having from one to two 5- to 6-membered mutually combined rings in the nucleus in which one of the rings has one to two hetero atoms of which one is a member of the group consisting of N, O and S, the second being nitrogen, and the remaining members of the nucleus being carbon atoms.

The following are examples of such nuclear aminoalkyl substituted heterocyclic compounds:



6-(β-aminoethyl)-2-methylbenzimidazole  
(German Patent 294,085 Beil. 25, 638)



5-(β-aminoethyl)imidazole (histamine)  
(Ber. 40, 3694)



6-(β-aminoethyl)benzimidazole  
(Beil. 25, I Supplement page 637, German Patent 294,085)



5-aminomethyl-1-methylimidazolone-(4)  
(Ber. 41, 2549)

3



4



60 These nuclear aminoalkyl substituted heterocyclic compounds are soluble in water and in alkaline developers, and may be used in specified amounts. Their solubility in water and in alkaline developers can be made appreciable by converting the base into a salt such as, for example, the sulfate, hydrochloride, carbonate, or carbamate. The sulfate and hydrochloride salts are readily prepared by the addition of a stoichiometrical quantity of dilute sulfuric acid and hydrochloric acid, respectively, and the carbonate or carbamate is prepared by introducing  $\text{CO}_2$  into an alcohol, benzene or ether solution of the base.

65

70

75

The most useful concentrations in black and

white developers range from about 1 gram to about 10 grams per liter of developer. In color developers the most useful concentrations range from about 2 grams to 5 grams per liter. Concentrations greater than 10 grams per liter of color developer have the tendency to distort the color balance of the color film.

In developing color images in multicolor photographic layers containing color formers fast to diffusion with a color developer containing a nuclear aminoalkyl substituted heterocyclic compound, the developing time is cut from 20-30 minutes to 2-10 minutes. All of the layers are simultaneously developed, and the dye images formed are of excellent quality.

The developing time with black and white developers, for instance, solutions of hydroquinone and p-monomethylaminophenol sulfate and the like, is also cut to about one-half without causing fog when such solutions contain a nuclear aminoalkyl substituted heterocyclic compound.

As illustrative of developing solutions containing such nuclear aminoalkyl substituted heterocyclic compounds, the following are given.

*Example I*

|                                   |       |        |
|-----------------------------------|-------|--------|
| Sodium hexametaphosphate          | grams | 1.0    |
| p-Methylaminophenol sulfate       | do    | 3.0    |
| Sodium sulfite (anhydrous)        | do    | 50.0   |
| Hydroquinone                      | do    | 6.0    |
| Sodium carbonate<br>(monohydrate) | do    | 40.0   |
| Potassium bromide                 | do    | 2.0    |
| Sodium thiocyanate                | do    | 2.0    |
| Potassium iodide                  | do    | 0.0035 |
| Furfurylamine                     | do    | 4.0    |
| Water to make                     | liter | 1      |

The foregoing developer on five minutes development at 20° C. of the usual black and white roll film gives a negative of good density and gradation after fixing and washing. The time required to develop the same film in the same solution but containing no furfurylamine ranges from 15 to 20 minutes.

The foregoing developing solutions containing the furfurylamine develops up to 1½-2 stops more speed in about 14 minutes as compared to the same developing solution containing no furfurylamine.

*Example II*

The following developer requires 30 minutes at 20° C. to give a satisfactory degree of color development for color paper:

|                                              |       |       |
|----------------------------------------------|-------|-------|
| Sodium hexametaphosphate                     | grams | 1.0   |
| Sodium sulfite (anhydrous)                   | do    | 2.5   |
| p-Amino-di(β-hydroxyethyl)aniline<br>sulfate | do    | 8.0   |
| Sodium carbonate (monohydrate)               | do    | 100.0 |
| Hydroxylamine hydrochloride                  | do    | 1.0   |
| Potassium bromide                            | do    | 1.0   |
| Water to make                                | liter | 1     |

By the addition of 4 grams of 5-aminomethyl-1-methylimidazolone [4] to the foregoing solution, a color paper of excellent color rendition is developed in about 10 minutes. Without the presence of said amine at least 30 minutes is required to give an acceptable print. Increasing the concentration of the amine further reduces the time of development.

The color photographic multilayer element utilized in the foregoing example consists of an

integral tri-pack emulsion coated on either the usual paper base, or a clear cellulose acetate or nitrate film base, or in some cases an opaque white film base. Each of the emulsion layers is sensitized to one of the primary colors of light, namely, blue, green, and red. The top layer is blue sensitive. A filter layer, yellow in color and blue absorbing, lies under the top layer. Below this filter layer lies a green sensitive emulsion layer, and below this a red sensitive emulsion layer. Each of the three silver halide emulsion layers contains dye forming compounds which unite during the development of a silver image in an aromatic amine developing agent to form a dye with the oxidation product of the developing agent. As silver is also formed during development, it must be removed after color development by treatment in a bleach, followed by a bath of sodium thiosulfate, as is well known in the art. A yellow dye is formed in the blue sensitive emulsion; a magenta dye is formed in the green sensitive emulsion; and a cyan dye is formed in the red sensitive emulsion. The combination of the dye images from these three printing primaries yields the color picture. Suitable methods for the preparation of multicolor emulsion layers have been described in the literature relating to color photography, and are, therefore, not described here.

*Example III*

A color developer similar to Example II but prepared with 5 grams per liter of p-aminomethyl(β-hydroxyethyl)aniline sulfate, and containing 4 grams of 2-aminomethylthiophene developed a multilayer color film of the reversal type, containing a color former fast to diffusion, in about 12 minutes at 20° C. whereas without the 2-aminomethylthiophene the color film is too low in maximum density for acceptable reproduction after 25 minutes.

The above examples are to be regarded as merely illustrative of the invention and not in any sense restrictive. It will be obvious to those skilled in the art that many modifications, such as substituting equivalent materials and varying the proportions of the materials used, are within the spirit and scope of the invention. The scope, therefore, of the invention is to be limited solely by the following claims.

I claim:

1. An alkaline photographic developer for silver halide emulsions comprising an aromatic silver halide developing agent and a nuclear aminoalkyl substituted heterocyclic compound, the nucleus of which is selected from the group consisting of one 5- to 6-membered ring and two 5- to 6-membered rings fused to each other one of said rings containing from 1 to 2 hetero atoms of which one is a member of the group consisting of N, O and S and the other is nitrogen, the remaining members of the nucleus being carbon atoms and the remaining nuclear substituents being selected from the class consisting of hydrogen, keto-oxygen, unsubstituted lower alkyl and unsubstituted monocyclic aryl hydrocarbon groups, and the nuclear aminoalkyl substituent group of which contains not more than 3 carbon atoms, and the salts of said amines.

2. An alkaline photographic developer for silver halide emulsions comprising an aromatic silver halide developing agent and furfurylamine.

3. An alkaline photographic developer for silver halide emulsions comprising an aromatic silver

halide developing agent and 5-aminomethyl-1-methylimidazolone[4].

4. An alkaline photographic developer for silver halide emulsions comprising an aromatic silver halide developing agent and 2-aminomethylthiophene.

5. In the development of a photographic negative, the step comprising the development of an exposed silver halide emulsion in an alkaline developer containing an aromatic silver halide developing agent for said emulsion and a developing accelerator consisting of a nuclear aminoalkyl substituted heterocyclic compound, the nucleus of which is selected from the group consisting of one 5- to 6-membered ring and two 5- to 6-membered rings fused to each other, one of said rings containing from 1 to 2 hetero atoms of which one is a member of the group consisting of N, O and S and the other is nitrogen, the remaining members of the nucleus being carbon atoms and the remaining nuclear substituents being selected from the class consisting of hydrogen, keto-oxygen, unsubstituted lower alkyl and unsubstituted monocyclic aryl hydrocarbon groups, and the nuclear aminoalkyl substituent group of which contains not more than 3 carbon atoms, and the salts of said amines.

6. In the development of a photographic negative, the step comprising the development of an exposed silver halide emulsion in an alkaline developer containing an aromatic silver halide developing agent for said emulsion and a developing accelerator consisting of furfurylamine.

7. In the development of a photographic negative, the step comprising the development of an exposed silver halide emulsion in an alkaline developer containing an aromatic silver halide developing agent for said emulsion and a developing accelerator consisting of 5-aminomethyl-1-methylimidazolone[4].

8. In the development of a photographic negative, the step comprising the development of an exposed silver halide emulsion in an alkaline developer containing an aromatic silver halide

developing agent for said emulsion and a developing accelerator consisting of 2-aminomethylthiophene.

9. A color forming photographic developer comprising a primary aromatic amino developing agent and a nuclear aminoalkyl substituted heterocyclic compound, the nucleus of which is selected from the group consisting of one 5- to 6-membered ring and two 5- to 6-membered rings fused to each other, one of said rings containing from 1 to 2 hetero atoms of which one is a member of the group consisting of N, O and S and the other is nitrogen, the remaining members of the nucleus being carbon atoms and the remaining nuclear substituents being selected from the class consisting of hydrogen, keto-oxygen, unsubstituted lower alkyl and unsubstituted monocyclic aryl hydrocarbon groups, and the nuclear aminoalkyl substituent group of which contains not more than 3 carbon atoms, and the salts of said amines.

10 10. A color forming photographic developer comprising a primary aromatic amino developing agent and furfurylamine.

11 11. A color forming photographic developer comprising a primary aromatic amino developing agent and 5-aminomethyl-1-methylimidazolone[4].

12 12. A color forming photographic developer comprising a primary aromatic amino developing agent and 2-aminomethylthiophene.

IVY V. RUNYAN.

#### REFERENCES CITED

35 The following references are of record in the file of this patent:

#### UNITED STATES PATENTS

| Number    | Name     | Date          |
|-----------|----------|---------------|
| 2,139,870 | Wilmanns | Dec. 13, 1938 |
| 2,289,367 | Kendall  | July 14, 1942 |
| 2,496,903 | Wasley   | Feb. 7, 1950  |
| 2,515,147 | Wasley   | July 11, 1950 |
| 2,541,889 | Runyan   | Feb. 15, 1951 |